

## UNITED STATES PATENT OFFICE.

BERTRAND S. SUMMERS, OF PORT HURON, MICHIGAN.

## PROCESS FOR MAKING PAPER HALF STOCK.

No Drawing.

Application filed January 24, 1920. Serial No. 353,824.

*To all whom it may concern:*

Be it known that I, BERTRAND S. SUMMERS, a citizen of the United States, residing at Port Huron, county of St. Clair, and State of Michigan, have invented a new and useful Process for Producing Paper Half Stock, of which the following is a specification.

My invention relates particularly to the production of a paper half stock suitable for the making of high grade white papers, such as cigarette paper, banknote paper, condenser paper, and the like. It is required that these papers shall be of absolute uniformity of texture, of a requisite degree of toughness, free from unreduced woody fibers and specks, which fibers and specks not only spoil the appearance of the paper but break its continuity, making it weak and useless for the purposes intended. Such papers have hitherto been made from linen stock, usually linen rags, and high grade mill waste. The supply of these materials in recent years has been much less than the demand, causing a great shortage in these papers and greatly increased price therefor.

There is, however, available a large quantity of flax straw resulting from the linseed and flax fiber industries. Many attempts have been made in the past to convert this material into paper half stock having the required characteristics. Owing to the physical and chemical peculiarities of flax straw, however, such attempts have not been successful, the problem being further complicated by the presence in such straw of foreign material, such as weeds.

It is well known that this flax straw and other straws contain ligneous matter as well as fibrous matters, and these two classes of matter have very different resisting powers to the action of agents adapted to reduce or remove the woody material. Flax is peculiarly characterized in that it contains not only the ligneous cellulose but also pecto cellulose. The fibrous portion of flax contains also cuto cellulose with strong waxy characteristics. The fibrous portion is very much less resistant to a reducing agent than is the ligneous portion. The ligneous portion of flax straw known as shive is one of the most resistant bodies in this respect that is known. All prior attempts, therefore, to use flax straw as a material for paper making have resulted in the presence in the paper of specks of foreign matter and un-

reduced shive, resulting in a paper of inferior quality both as to appearance and strength and useless for the purposes to which high grade linen papers are applied. To my knowledge papers which have hitherto been produced from these straws, while sometimes of good color so far as the fibrous portion is concerned, have contained a large element of unreduced matter, which weakens the paper, while any attempt to reduce this matter has resulted in the destruction of the fibrous matter, making it impossible to make a high class sheet. To my knowledge, therefore, although vast supplies of material have been available, it has hitherto been impossible to use them.

In carrying out my invention, I treat the straws having the characteristics above described by first removing therefrom such of the ligneous material as may be done by the usual breaking and dusting process. This partially cleaned material contains a considerable portion of the shive together sometimes with a quantity of weedy material. It has been found impracticable to remove all such material by mechanical operation alone. I then subject this material to the usual boiling off process which results in a partial reduction of the woody material. For this boiling off may be employed any of the lime or alkaline materials commonly used for this purpose. The material may then, if desired, be washed in a suitable acid. I then subject the material to a very strong chemical reaction, this reaction having the peculiar property of intensely attacking the woody or foreign material associated with the fiber without injuring the strength or integrity of the fibrous portion. For this purpose I employ a very strong solution of calcium hypochlorite, commonly known as a bleaching powder. This hypochlorite is dissolved in water and allowed to settle. A sufficient quantity of hypochlorite is introduced into the water to bring the solution to a density of 4 to 6 Twaddle, although this may be varied to suit the requirements of the material to be treated. The calcium hypochlorite solution is allowed to settle and drained off. I then introduce into this solution sodium bicarbonate in excess. I preferably make a saturated solution of sodium bicarbonate and introduce the same into the calcium hypochlorite solution. By adding an excess of the sodium bicarbonate over the quantity required to completely precipitate

the calcium hypochlorite a condition results whereby a perfectly clear solution is obtained. This clear solution containing sodium hypochlorite and sodium bicarbonate is then decanted or pumped from the precipitated calcium carbonate and is introduced into the vessel containing the material to be treated. This vessel is preferably arranged so that the material is kept in 10 agitation. For this purpose an ordinary paper maker's beating engine may be employed, in which the metal parts are such as will not be acted upon by the chlorine compounds to the detriment of the stock. 15 The time required to complete the reduction of the material varies considerably with the amount of woody matter contained therein. Material also that has been weather damaged and darkened requires somewhat 20 longer time than straw that has not been thus discolored. The reduction usually requires from three to eight hours, depending upon the conditions above indicated.

When the reduction is complete, the material is thoroughly washed and preferably treated with a small amount of any chemical capable of destroying any remaining chlorine products which may be retained by the material, such, for instance, as sodium bisulphite. When the stock is again washed, it may be used directly for paper making or dried in the form of half stock. It will be observed that in carrying out my process, I have used materials which may have 30 hitherto been employed in the bleaching of textiles. It will be observed, however, that I employ greatly different proportions and much higher concentrations when reducing woody materials.

40 In practicing my invention, I introduce a suitable excess of the sodium bicarbonate and not only transform the calcium hypochlorite into sodium hypochlorite but keep considerable sodium bicarbonate in solution in the bath. I have noticed that to avoid undue evolution of gases, it is preferable to introduce sodium bicarbonate in a dissolved condition, and gradually. In fact, if it is desired to introduce solid sodium bicarbonate, no agitation of the bath should take place while such introduction is being practiced.

It results from my process as carried out in the manner above described with fibrous 55 material containing woody material and foreign matters, that an intense chemical bath is formed, which has very great reduction powers toward these woody materials without unduly attacking the fibrous portion. In fact, this reduction effect is so noticeable that in the course of a few hours the woody matter entirely disappears with proper management of the bath, while fibrous matter remains in practically 60 full strength and proper color. It will

be apparent to any one skilled in the art that a bleaching effect is the necessary result of this reaction, but the primary effect is to reduce or destroy the woody and foreign matter, leaving a paper maker's 70 material of high quality, of practically pure cellulose and containing no defective matters.

I have produced by this process from flax straw, treated as above described, paper 75 half stock of the highest quality, entirely suitable for the production of the high class papers required for the purposes hereinbefore mentioned, and this without subjecting the straw to any retting process. I believe that I am the first in this art to accomplish this result, such papers having hitherto been made only from linen rags and other high class material.

Having now described my invention and 85 what I desire to secure by Letters Patent, I claim:

1. The herein described process which consists in adding to a strong solution of calcium hydrochlorite a saturated solution 90 of sodium bicarbonate, removing the supernatant liquid, and subjecting a woody and fibrous material to the action of this liquid.

2. The herein described process, which consists in adding to a strong solution of calcium hypochlorite sodium bicarbonate in excess, removing the supernatant liquid, and subjecting woody and fibrous material to the action of this liquid.

3. The herein described process of making 100 paper half stock, which consists in treating a woody and fibrous material to a sufficiently concentrated solution containing chlorinous material in active condition together with an alkaline bicarbonate, substantially as 105 described.

4. The herein described process of making paper half stock, which consists in treating a woody and fibrous material to a sufficiently 110 concentrated solution of hypochlorite, said solution containing a material capable of liberating carbon dioxide.

5. The herein described process of making paper half stock, which consists in adding 115 to a sufficiently concentrated solution of calcium hypochlorite an excess of sodium bicarbonate, withdrawing the supernatant liquid, and subjecting fibrous straws containing woody material to the action of this liquid, substantially as described.

6. The herein described process of making paper half stock, which consists in adding to a sufficiently concentrated solution of calcium hypochlorite an excess of alkaline 125 bicarbonate, withdrawing the supernatant liquid, and subjecting fibrous straws containing woody material to the action of this liquid, substantially as described.

7. The herein described process, which 130 consists in mechanically cleaning flax straw,

or the like, boiling out the straw thus partially cleaned, and then subjecting the straw to the action of a liquid resulting from the introduction into a sufficiently concentrated 5 solution of calcium hypochlorite of an excess of sodium bicarbonate.

8. The herein described process, which consists in mechanically cleaning flax

straw, or the like, boiling out the straw thus partially cleaned, and then subjecting the straw to the action of a liquid resulting from the introduction into a sufficiently concentrated solution of chlorinous matter in an active condition of an excess of alkaline bicarbonate.

BERTRAND S. SUMMERS.